

## 1

2,734,030

## MIXED SOAP-COMPLEX GREASE COMPOSITIONS

Eric O. Forster, Hillside, and Joseph P. Hamer, Somerville, N. J., assignors to Esso Research and Engineering Company, a corporation of Delaware

No Drawing. Application February 20, 1953,  
Serial No. 338,148

6 Claims. (Cl. 252—39)

This invention relates to lubricating grease compositions, and particularly to lubricating grease compositions having outstanding high temperature and structure stability properties. More particularly the invention relates to a mixed soap grease containing combined therein a minor amount of a low molecular weight salt in the form of a complex with the mixed soap.

The preparation of calcium base grease is old in the art and is well described in the patent literature. Such greases are excellent in structure, water resistance, and appearance. However, the high temperature properties of calcium greases are very poor. This is due to the necessity of maintaining a certain amount of water in the grease itself. At temperatures above about 200° F. the water of formulation is driven off and the grease structure breaks down, resulting in separation of the oil.

It has recently been found, and is described in detail in copending application, Serial Number 301,194, filed July 28, 1952, now Patent No. 2,708,659, of which this application is a continuation-in-part, that a calcium base grease having all the advantages of water resistance and characteristic structural stability of the calcium greases, and having, in addition, excellent high temperature properties may be prepared by combining with the calcium soap of the prior art varying amounts of a soap of a metal selected from the group consisting of magnesium, barium, and strontium. Certain processing steps are necessary for the preparation of the greases described in the copending application which are described in detail therein.

It has now been found, and forms the object of this invention, that these mixed base greases may be improved in structure stability and high temperature performance by complexing with the mixed base soap, a metallic salt of a low molecular weight acid, preferably one having from one to six carbon atoms. The incorporation of a salt of a low molecular weight acid in the complex form with the high molecular weight acid soap gives better high temperature performance and increased structure stability.

*The mixed soap base*

The mixed soap base which serves as the thickening agent for the improved grease compositions of this invention comprises a mixture of the calcium soap of high molecular weight fatty acids and a soap of a metal selected from the class consisting of barium, strontium, and magnesium.

The high molecular weight fatty acids operable in preparing the mixed soaps may be selected from the well known grease-making materials which include oleic acid, stearic acid, hydroxy stearic acid, hydrogenated fish oil acids, glycerides, tallow, beef fat, and the like, including mixtures of the above in any proportion. Fatty acids having carbon chain lengths of from about 12 to 24 carbon atoms, and mixtures thereof, are especially preferred. Hydrogenated fish oil acids are examples of these preferred acids.

## 2

The calcium soap must be present in amounts ranging from about 2.5% to about 15.0% by weight, based on the weight of the finished formulation. The amount of the soap of the second metal used is such that the mol ratio of the calcium soap to the second soap is within the range of from 8:1 to 1:8, with a mol ratio within the range of from 8:1 to 3:1 being especially preferred. The amount of the combined soaps present will depend somewhat upon the desired final consistency of the product. Ordinary usage would call for a grease composition according to the instant invention containing from about 5.0% to 30.0% by weight of the combined soap, with a range of from 10.0% to 20.0% being especially preferred.

*The complexing salt*

The low molecular weight organic acid salt which is used to form the complex with the mixture of high molecular weight acid soaps can be derived from any number of organic acids having from one to six carbon atoms. The use of acetic or propionic acid is desirable, with acetic being preferred and used in the preferred embodiment. The metal used may be selected from the class consisting of calcium, barium, magnesium, or strontium, with the former being preferred. The salt may be added to the soap mixture in the form of a slurry of the dry salt and oil, in the form of the dry salt, or it may be prepared in situ. The amount of the salt used will be such as to result in a mol ratio of the total soap to salt of about 0.70 to about 1.2. Mol ratios of greater than 1.2 or less than 0.7 will not produce the results desired. A mol ratio of mixed soaps to the salt of from 0.75 to 1.0 is especially preferred.

*The lubricating oil base*

The lubricating oil which is utilized as a dispersant for the soaps in preparing the greases of invention may be selected from a wide variety of lubricating oils. A mineral lubricating oil preferably of naphthenic origin may be chosen as the base. It should have a viscosity within a range of from about 40 SUS at 100° F. to about 4000 SUS at 100° F. As in the preparation of most grease compositions, the mineral oil chosen should be that lubricating oil which would be used to furnish proper lubrication if a liquid oil could be used. It is preferred to use a mineral oil having a viscosity of from about 200 to 1500 SUS at 100° F. to formulate the greases of the preferred embodiment.

Although a mineral lubricating oil, such as a conventionally refined distillate, is preferred for the preparation of the improved greases of invention, a synthetic oil may also be utilized as the dispersing agent. Although a synthetic lubricant of the ester type is preferred, such as the esters of dibasic acids and long chain alcohols, other well known synthetic lubricants may be used. Complex esters made from dibasic acids, glycols, and alcohols, may be used, as may the polymerized glycol esters, glycol ethers, polymerized olefins, alkylated aromatics, polymerized silicones, formals, mercaptals, and the like. The only requisite for the oil base is that the one chosen be one that will furnish the desired lubrication when utilized as a grease.

*Method of preparation*

The same two process limitations described in detail in copending application, Serial Number 301,194, pertain to the manufacture of the instant grease formulations; namely, the dispersion of the calcium soap prior to the dispersion of the second soap and heating the total formulation to a temperature of at least 350° F. after dehydration. The exact reasons are not known why these limitations are critical, but again it is believed that the solu-

tion of the calcium soap in the oil aids in the dispersion of the second soap and that above 350° F. there is a phase transition of the soap mixture which produces a new arrangement of molecules that is stable both at low and elevated temperatures. It is also essential to raise the mixture to these high temperatures in order to form the complex of the mixture of soaps and the salt, a complex which is believed to be largely responsible for the excellent high temperature and shear stability properties obtained.

The method of manufacture of the greases of this invention may be generally described as follows.

The mixture of high molecular weight soap is prepared first by saponifying a part of the saponifiable material with calcium hydroxide in the presence of one third of the total amount of base oil. Then barium hydroxide is added in the form of a slurry or as a dry powder to saponify the remainder of the fatty acid. Calcium acetate or barium acetate, as the case may be, is then added as a dry powder or as a water or oil suspension, or if desired it may be formed in situ. The soaps are dehydrated and heated to above about 350° F. The remainder of the base oil is then added and the mixture heated to 450° F. to 480° F. At that temperature the mixture is a homogeneous semi-solid mass. While stirring continuously the grease is cooled until the temperature is in the neighborhood of 150° F. The stirring is then stopped, and the grease cooled to room temperature. It is then thoroughly worked, as by passing through a Morehouse mill or other well known working device.

To illustrate the concept of this invention and to point out the advantages of the new grease formulations over those of the prior art, nine grease samples were prepared. The first preparation was carried out in accordance with the literature and a complex of calcium soap and a calcium salt was prepared. The second and third formulations were prepared as described in Serial Number 301,194, the copending application mentioned above. Examples 4 through 9 were prepared in accordance with the inventive concept as described in detail above. These grease samples were submitted to the standard grease inspection tests including the penetration tests, the determination of the neutralization numbers and the resistance to boiling water. The data obtained on these 9 greases are set out in table form below.

high temperature properties could be improved. This is illustrated by the data of Examples 2 and 3. The data on Examples 4 through 9, prepared in accordance with the instant invention show both excellent high temperature properties and excellent structural stability, at various soap concentrations and complex proportions. It seems clear that the combination of an alkaline earth metal salt of low molecular weight acids with a mixture of two alkaline earth metal soaps of high molecular weight fatty acids produces a grease that is superior to either one formed from a mere combination of low molecular weight salts and a single high molecular weight soap, or a mixture of two high molecular weight soaps alone. Calcium acetate seems to be the most effective complexing agent, with barium acetate being very acceptable.

Other additive materials, such as oxidation inhibitors, color agents, stringiness or tackiness agents and the like may also be used in preparing the greases of invention. These agents are ordinarily added after the heating has been completed and before the grease has cooled completely.

To reiterate briefly, the instant invention relates to superior high temperature lubricating grease compositions that are prepared by complexing with a mixture of the metallic salts of high molecular weight fatty acids, a metallic salt of a low molecular weight acid. Specifically, the alkaline earth metals are desired, such as calcium, barium, strontium, and magnesium. Particularly desired and contemplated in the preferred embodiment are the mixtures of the calcium and barium soaps of high molecular weight fatty acids complexed with the calcium salt of a low molecular weight acid having from one to six carbon atoms. Mol ratios of from 8:1 to 1:8 of calcium soap to barium soap is contemplated, with the total soap mixture comprising from about 5.0 wt. percent to 30.0 wt. percent of the total formulation. The low molecular weight salt is added in amounts such that there is present a mol ratio of total soap to salt of from 0.70 to 1.2, preferably from 0.75 to 1.0. It is also essential that the calcium soap be dispersed prior to the dispersion of the barium soap in the mineral oil.

What is claimed is:

1. A lubricating grease composition having outstanding high temperature properties which comprises a lubri-

TABLE

| Example No.                                         | 1          | 2          | 3          | 4          | 5          | 6          | 7          | 8          | 9          |
|-----------------------------------------------------|------------|------------|------------|------------|------------|------------|------------|------------|------------|
| High Mol Wt. Soap Type                              | Ca         | Ca/Ba      | Ca/Ba      | Ca/Ba      | Ca/Ba      | Ca/Ba      | Ca/Ba      | Ca/Ba      | Ca/Ba      |
| High Mol Wt. Soap, Mol Ratio                        | 1          | 8/1        | 4/1        | 8/1        | 4/1        | 4/1        | 4/1        | 4/1        | 8/1        |
| Percent Saponif. Material                           | 10         | 17         | 10         | 10         | 10         | 12.5       | 12.5       | 10         | 10         |
| Low Mol Wt. Salt Type                               | Ca-Acetate | Ca-Acetate | Ca-Acetate | Ca-Acetate | Ca-Acetate | Ca-Acetate | Ca-Acetate | Ba-Acetate | Ba-Acetate |
| Percent Low Mol Wt. Salt                            | 3          | 3          | 3          | 3          | 3          | 3          | 2          | 3          | 3          |
| Mol Ratio:                                          |            |            |            |            |            |            |            |            |            |
| Low Mol Wt. Salt                                    |            |            |            |            |            |            |            |            |            |
| High Mol Wt. Soap                                   | 1.07       |            |            | 1.07       | 1.07       | 0.86       | 0.57       | 0.66       | 0.66       |
| Dropping Point, ° F.                                | 452        | 308        | 282        | +520       | +520       | +520       | 346        | 414        | 394        |
| Penetration in mm./10:                              |            |            |            |            |            |            |            |            |            |
| Unworked                                            | 320        | 219        | 286        | 268        | 258        | 175        | 175        | 375        | 318        |
| Worked (10,000 strokes in ASTM Worker) <sup>1</sup> | 430        | 272        | 325        | 368        | 329        | 243        | 280        | 322        | 345        |
| Neut. Number, Percent NaOH                          | 0.12       | 0.73       | 0.13       | 0.22       | 0.28       | 0.30       | 0.32       | 0.47       | 0.25       |
| Resistance to boiling water                         | fair       | excel.     | excel.     | excel.     | excel.     | excel.     | excel.     | excel.     | excel.     |

Typical Composition of a Sample (In weight percent):  
10% Hydrogenated Fish Oil Acids  
3% Calcium acetate

1.28% Ba(OH)<sub>2</sub>·8H<sub>2</sub>O  
1.24% Ca(OH)<sub>2</sub>  
84.48% Diol 70<sup>2</sup>

<sup>1</sup> Using plate with small holes.

<sup>2</sup> Acid treated coastal distillate having a viscosity of 70 S. U. S. at 210° F.

The data of the table above point out the advantage of the greases prepared in accordance with the inventive concept. It will be noted that the calcium-calcium acetate complex grease of the prior art, Example 1, has excellent high temperature properties, but that it fluidizes after 10,000 strokes with the fine hole worker indicating a lack of structural stability. The Ca/Ba grease of Serial No. 301,194 has excellent structural stability but its

cating oil thickened with from about 5.0 to 30.0% by weight, based on the weight of the total composition, of a complex formed from a mixture of a calcium soap and a second soap selected from the group consisting of barium, strontium and magnesium soaps of high molecular weight fatty acids and a metal salt of a low molecular weight carboxylic acid having from one to six carbon atoms, said metal being selected from the

group consisting of calcium, barium, magnesium and strontium, the calcium soap being present in an amount ranging from about 2.5 to 15.0% by weight, based on the weight of the total composition, the mol ratio of said calcium soap to said second soap being about 8:1 to 1:8, the mol ratio of said mixture of soaps to said metal salt being within the range of about 0.70 to 1.2, said complex being formed by first dispersing the calcium soap in the lubricating oil, then dispersing the second soap and said metal salt, and heating the resulting mixture to a transition temperature from about 350° to 480° F.

2. A lubricating grease composition according to claim 1 wherein the lubricating oil is thickened with from about 10.0 to 20.0% by weight of the complex, based on the weight of the total composition, the mol ratio of said calcium soap to said second soap is between about 8:1 to 3:1, and the mol ratio of said mixture of soaps to said metal is between about 0.75 to 1.0.

3. A lubricating grease composition according to claim 1 wherein said fatty acid contains about 12 to 24 carbon atoms.

4. A lubricating grease composition according to claim 1 wherein said second soap is a barium soap.
5. A lubricating grease composition according to claim 1 wherein said fatty acid is hydrogenated fish oil acid.
6. A lubricating grease composition according to claim 1 wherein said salt is calcium acetate.

References Cited in the file of this patent

UNITED STATES PATENTS

|    |            |                   |               |
|----|------------|-------------------|---------------|
| 10 | Re. 23,082 | Zimmer et al.     | Jan. 25, 1949 |
|    | 2,070,781  | Brunstrum et al.  | Feb. 16, 1937 |
|    | 2,197,263  | Carmichael et al. | Apr. 16, 1940 |
|    | 2,389,523  | Leyda             | Nov. 20, 1945 |
|    | 2,417,429  | McLennan          | Mar. 18, 1947 |
| 15 | 2,417,433  | McLennan          | Mar. 18, 1947 |
|    | 2,495,651  | Butcosk           | Jan. 24, 1950 |
|    | 2,513,680  | Shott et al.      | July 4, 1950  |
|    | 2,553,423  | Shepard           | May 15, 1951  |
|    | 2,564,561  | Carmichael et al. | Aug. 14, 1951 |
| 20 | 2,583,394  | Shott et al.      | Jan. 22, 1952 |